

Patented Mar. 1, 1927.

## UNITED STATES PATENT OFFICE.

EDWARD F. KENNEY, OF BETHLEHEM, PENNSYLVANIA.

## HEAT TREATMENT OF STEEL.

No Drawing.

Application filed April 23, 1926. Serial No. 104,224.

REISSUED

My invention relates to the heat treatment of worked steel objects, those particularly, such as railway rails and wheels, as have different degrees of thickness.

It consists essentially in hardening the object by rapidly cooling it from a temperature above to a temperature below the critical range, and then, before the object has cooled to a temperature as low as the blue-heat zone, maintaining it at a temperature between the critical range and the blue-heat zone to thoroughly equalize the temperature, after which it may be cooled to atmospheric temperatures.

In order that a steel object, such as a rail, has the proper combination of hardness and toughness, it is essential that it be uniformly heated above the critical range and then rapidly cooled to a temperature below such

range. In the further cooling of the object a temperature range is passed through in which the metal is more or less plastic and thereby capable of withstanding stresses without rupture or serious strains. When the temperature, however, has dropped as low as the blue-heat zone, this plasticity is largely lost.

Now if an object, such as a rail, having some portions substantially thinner than others, after being cooled through the critical range, were allowed to further cool, uncontrolled, to atmospheric temperatures, naturally the thinner portions would cool much more rapidly than the thicker and would enter the blue-heat zone much sooner. At this stage the plasticity of the thinner portions would be much reduced, while the thicker portions at a substantially higher temperature would still be in the plastic stage. Consequently, upon further cooling of the thicker portions with resulting contraction, the thinner portions of the metal now being low in plasticity, stresses are set up which produce serious strains and even rupture.

To control the cooling and thereby prevent this condition is the purpose of my invention.

My invention may be best illustrated by setting forth several specific examples.

Rails of the following composition—Carbon .63 to .87, manganese .60 to .90, phosphorus .03, sulphur .05, and silicon .15 to .25 were quenched in water for about thirty seconds from a temperature about 1750° F.,

bringing the temperature down to about 725° F., the cooling thus being from a temperature above the critical range to one below it but above the blue-heat range. The rails were then charged immediately into a furnace maintained at 1000° F. They were kept at this temperature one hour and then removed from the furnace and allowed to cool in the air. Under the drop test these rails were tougher than the regular rail which has not been quenched and they showed no sign of ruptures.

Rails of the following composition—

| Carbon. | Manganese. | Phosphorus. | Sulphur. | Silicon. |
|---------|------------|-------------|----------|----------|
| .62     | 1.32       | .023        | .044     | .16      |
| .72     | 1.43       | .022        | .042     | .19      |
| .68     | .72        | .023        | .062     | .13      |
| .72     | .79        | .024        | .060     | .19      |
| .74     | .69        | .023        | .049     | .26      |
| .86     | .81        | .023        | .057     | .22      |

were also treated by quenching from a temperature of 1550° F., the quenching stopped before the blue-heat zone was reached, and immediately equalized at 900° F.

Extensive tests were made upon these rails, including drop tests, Brinell hardness tests, Izod impact tests, and macroscopic and microscopic examinations. The physical properties were greatly improved and no signs of internal ruptures found.

On the other hand, when rails of the same compositions were quenched in the same way but without being given the equalization treatment between the critical range and the blue-heat zone, the metal structure was found to be badly ruptured.

For example, some of the rails were quenched from a temperature of 1750° in water for 2 minutes, bringing them nearly to atmospheric temperature. These rails broke into a number of fragments before they were removed from the quenching tank.

Again, rails were quenched in water from a temperature of 1750° F. for 30 seconds and then allowed to cool in air, there being no equalization treatment. These rails cracked in cooling and when cut up and examined macroscopically and microscopically were found to be badly ruptured internally as well as externally.

It is economically advantageous to carry out my process in connection with the mechanical working. For example, in the manufacture of rails after leaving the rail mill

- and while still in a heated condition, they are passed into a suitable equalizing chamber where they are brought to a uniform temperature above the critical range. This equalizing chamber will, of course, be maintained at the desired temperature by any suitable heating means. After being equalized the rails are quenched to a temperature below the critical range but above the blue-heat zone. Without allowing them to cool they are immediately charged into a furnace kept at a temperature preferably between 800° and 1100° F. and kept there until the temperature is thoroughly equalized.
- 10 Then, after straightening, they are allowed to cool to atmospheric temperature. Of course, all the details here mentioned are not always essential. For example, the equalizing before the quenching may be omitted.
- 15 The choice of temperature for equalizing, after the quenching operation, varies with the particular combination of hardness and toughness desired.
- 20 What I mean by the "blue-heat zone", as this expression is used in this disclosure, is that range of temperatures, below the critical range where steels in heating markedly increase in tensile strength and the elastic limit, and also markedly decrease in ductility. At temperatures, within this range, most steels when exposed to air take on a blue color, due to oxidation, but since, with some steels, this color is not readily ap-

parent, I do not wish to be limited to the 35 color as a means of determining or defining this zone.

By the expression "critical range" I mean that temperature range through which the steel must be cooled to effect a hardening 40 thereof. This range will vary with the particular composition of the steel, the various ranges according to different carbon contents being in the common nomenclature A<sub>1</sub>, A<sub>3</sub><sub>—2</sub>, and A<sub>3</sub><sub>—2</sub><sub>1</sub>. 45

Having thus described the invention what I claim as new and desire to secure by Letters Patent is:

1. The process of heat treating a steel object which consists in rapidly cooling it from 50 a temperature above to a temperature below the critical range, then equalizing at a temperature below the critical range but before the object has cooled to the blue-heat zone, and then cooling to atmospheric tempera- 55

2. The process of making a steel object of irregular shape, consisting in mechanically shaping the steel, in cooling rapidly from 60 above to below the critical range before the object has lost the heat incidental to shaping, equalizing at a temperature between the critical range and the blue-heat zone before the object has cooled to the blue-heat zone, and cooling to atmospheric temperature. 65

In testimony whereof I hereunto affix my signature this 20th day of April, 1926.

EDWARD F. KENNEY.